

March 8, 1960

W. S. NORMAN

2,927,877

HEAT EXCHANGER

Filed June 1, 1954

3 Sheets-Sheet 1



INVENTOR

William S. Norman

By Watson, Cole, Grindle &  
Watson

ATTORNEYS

March 8, 1960

W. S. NORMAN  
HEAT EXCHANGER

2,927,877

Filed June 1, 1954

3 Sheets-Sheet 2



INVENTOR  
William S. Norman  
By Watson, Cole, Grindler  
Watson  
ATTORNEYS.

March 8, 1960

W. S. NORMAN

2,927,877

Filed June 1, 1954

## HEAT EXCHANGER

3 Sheets-Sheet 3



INVENTOR

William S. Norman

By Watson, Cole, Grindle &  
Watson

ATTORNEYS

1

2,927,877

## HEAT EXCHANGER

William Stephens Norman, Hoole, Chester, England, assignor to C. D. Patents Limited, London, England, a British company

Application June 1, 1954, Serial No. 433,773

Claims priority, application Great Britain January 14, 1949

2 Claims. (Cl. 154—75)

The present application is a continuation-in-part of my prior similarly entitled application Serial No. 120,480 filed October 10, 1949, now abandoned.

This invention relates to improvements in heat exchangers which are constructed or substantially constructed of elementary carbon. Elementary carbon possesses specially advantageous properties for the exchange of thermal energy between fluids, especially where one or both of the fluids is an active chemical substance with strongly corrosive or solvent action. In general, metallic elements and alloys have high thermal conductivity, but with the exception of the noble metals they have poor resistance to attack by corrosive chemical agents. Non-metals, metallic oxides, silicates and other materials commonly used for handling corrosive liquids and gases have poor thermal conductivity and are therefore inappropriate for use as materials of construction for heat transfer apparatus. They also have in general poor mechanical strength. Elementary carbon has thermal conductivity of the same order as the metallic elements but is very much more resistant to corrosion than those metals which are freely and cheaply available for constructional purposes. On the other hand, carbon exhibits its greater strength under compression and is brittle. It is therefore not well adapted to the construction of tubular heat exchangers of the kind commonly used when the material of construction is metallic. The term carbon as used in this specification refers to all forms of carbon in which the molecular structure is predominantly of carbon-carbon linkages. This includes what is commonly called amorphous carbon and also graphite, whether natural or produced by the subjection of amorphous carbon to high temperatures including such partially graphitised carbons as are produced in the temperature range from 1700 to 2500° C. It also includes material predominantly carbon in which carbon particles are bonded by some organic or inorganic binding agent.

There are many industrial processes in which heat exchangers are used to transfer heat from one moving fluid to another moving fluid, the effect being to increase or decrease the temperature of any one fluid according to whether it enters the heat exchange system at a lower or at a higher temperature than that of the other fluid. One type of heat exchanger in common use comprises an assembly of plates and is known as the plate type. Another type, which is perhaps in most common use today, is the tubular type, one example of which comprises a number of parallel tubes each about 6 feet long located between two headers. A fluid is made to flow through the tubes, and the tubes are traversed externally by the other fluid, the effect of which is to heat or to cool, as the case may be, the fluid passing within the tubes.

Owing to the cheapness of metal tubes and their high thermal conductivity and mechanical strength even with walls as thin as  $\frac{1}{32}$ ", it is customary to make tubular heat exchangers of metal wherever operating conditions permit. There are however circumstances in which

2

metal conduits are inappropriate; for example, one or other of the fluids may have some action on metal such as a corrosive action, or the metal may react upon one of the fluids either directly or catalytically. Hence for some purposes tubular heat exchangers are made from carbon or graphite. They are necessarily more expensive than those made from the commoner metals, and they are much more susceptible to damage under transport, handling, and operating conditions. Moreover, for adequate mechanical strength, the wall thickness of the tubes may have to be three or more times that of metal tubes of the same internal diameter, although it is obvious that the thinner the wall the better the heat transfer.

It is known to make a heat exchanger by forming passages through a metal block, one fluid flowing through a set or group of parallel conduits while the other fluid flows through another set or group of parallel conduits adjacent to and crossing the first set or group.

In metal heat exchangers this block principle of construction does not appear to have achieved any commercial success, probably because the metal tubular type was cheaper and of quite adequate strength.

One main object of this invention is to produce a heat exchanger unit composed of carbon or graphite in a strong, tough and coherent form. Another object is to provide specific means of producing a heat exchanger unit of the appropriate type. A third object is to provide physical methods of building or making the foraminous body.

The invention provides a method of manufacturing a low porosity carbon heat exchanger body comprising assembling a plurality of carbon plates to form a block, said plates being grooved to provide passages traversing said block, impregnating the assembled plates and therebetween with a liquid organic resin, and heat-hardening said resin to reduce the porosity of the plates and bond them together.

The carbon plates can be composed of carbon produced from finely sub-divided bituminous coal by the process described in U.S. Patent No. 2,461,365.

In an alternative form the carbon plates are made from coal or coke or a mixture consisting predominantly of coal or coke and a minor proportion of a carbon-producing binder, such for example as pitch, after which the plates are fired to carbonize said binder and impart strength and toughness to the fired plates.

In both cases if the final temperature of the heating operation does not exceed 1600° C. the product will be practically pure carbon and if the final temperature is increased to that necessary for electrographitization, say 2250° C. or above, the carbon will be in the form of graphite. Either form of carbon may be employed in this invention.

There are various ways in which the heat exchanger block with its cross-flow passages may be produced or built up.

In one method flat plates with the appropriate grooves may first be formed as described hereinafter and the required number of such plates may be cemented together in the required relation to one another to form the complete foraminous block. Thereafter the block is impregnated with a liquid organic resin. Alternatively, the cementing or bonding operation may be conducted simultaneously with an impregnating operation.

Headers for introduction and discharge of the fluids may themselves be formed of carbon or graphite parts moulded and fired by techniques analogous to those above referred to. The headers may be joined to the body by a carbonaceous cement and may be impregnated. The headers may be of metal if the metal is not affected by the heat exchange fluids.

A block type of heat exchanger comprising a 12" cube with approximately 250  $\frac{3}{8}$ " holes in each direction has the same heat transfer surface as 15 tubes, each 6' long and of 1" internal diameter.

The liquid organic resin may be converted into carbon. Thus it may consist of a mixture of furfural with concentrated sulphuric acid (with or without finely divided carbon) or it may be an artificial resin which when raised to a high temperature is carbonised.

The process of simultaneous cementing and impregnation may consist of clamping the unimpregnated plates together in the correct alignment and then impregnating by evacuation, submerging in a liquid resin and applying pressure to force the liquid into the pores. The liquid resin having been poured out of the passages the resin (which has penetrated into the joints between adjacent carbon plates) is cured or hardened by baking and a strong and permanent bond is formed between the plates.

Alternatively the carbon plates may be cemented together before the above impregnating procedure is followed.

In an alternative method of impregnating, the liquid resin is supplied under pressure to passageways traversing the assembled block, draining and curing following. This procedure may be followed by the vacuum impregnation described above.

The liquid organic resin may be any suitable resinous material which in the unpolymerised or partly polymerised state is sufficiently fluid to permeate the porous voids in the carbon, and which can be polymerised to form a hard cement after the impregnation. Suitable resins are described in the examples given hereinafter.

In carrying out the method of the invention the following points are of practical importance:

(a) Before impregnation the assembled plates should be thoroughly dried (e.g. by heating for at least an hour at 125° C.).

(b) It is necessary to ensure that the carbon plates shall be held firmly together throughout the impregnation and curing steps and especially the latter, bearing in mind the differential expansion of the carbon and the metal bolts of the cover plates when heat is applied. It is also desirable that the completed heat exchanger body when ready for use shall be under compression between the cover plates. Thus, when simultaneous bonding and impregnation are performed it is desirable that the bolts shall be tighter than when pre-cementing is used, since in the latter case the cement is sufficient to hold the carbon plates together during polymerisation of the resin.

A suitable final torque loading for each of four 1 inch diameter corner bolts for the cover plates of a heat exchanger block comprising a 15 inch cube is 80 ft.-lbs., the block being ready for use at this loading. In the manufacture of the block by simultaneous bonding and impregnation, it has been found that a suitable bolt loading as soon as the plates are assembled is one of at least 175 ft.-lbs. and that no adjustment of the bolts need be made until after polymerisation when adjustment is made to the required loading of 80 ft.-lbs. In using pre-cementing, the carbon plates are preferably held with the bolts adjusted to hand tightness until the cement has hardened, when the bolt loading is adjusted to 80 ft.-lbs. Impregnation and curing follow and thereafter any necessary final adjustment of the bolts to ensure a loading of 80 ft.-lbs. is made.

(c) The viscosity of the liquid impregnating resin should preferably be in the range of 30 to 100 centipoises. (Between 30 and 40 centipoises is usually most suitable.)

(d) In vacuum impregnation, the vacuum should be the highest practicable. The vacuum should not if avoidable be above 10 mm. of mercury absolute and is preferably about 3 mm. of mercury absolute.

(e) The vacuum treatment should generally be for at least one hour.

(f) The pressure applied to force the liquid into the pores is suitably about 50 lbs. per square inch but higher pressures may be used.

(g) The time of immersion under pressure should usually be for at least one hour.

(h) Before polymerisation excess resin should be permitted to drain from the block and ample time should be allowed for this (e.g. about 12 hours).

(i) The heating of the block for polymerisation of the impregnating resin should be done at a rate such as to avoid loss of resin. If the block is heated to high temperatures too rapidly, resin exudes to the surface of the block thus weakening the resulting structure and impairing its heat transfer properties. The temperature should be slowly and gradually increased to the required final value. A suitable heating schedule for a cashew nut shell resin is:

20 24 hours at 50° C.  
36 hours at 100° C.  
24 hours at 120° C.

(j) To ensure sufficiently low porosity, two separate impregnating stages may be employed, the second impregnation following the curing of the resin of the preceding stage. Both impregnating stages may involve vacuum treatment, or one stage may involve vacuum treatment while in the other stage liquid resin is forced into the passages of the block. Different resins may conveniently be used in the two stages.

(k) The guide to whether impregnation has been adequate is whether the heat exchanger body leaks when tested (e.g. by immersion in water and the supply of pressure air to the passages in the body).

It is preferred that each carbon plate has on one side a first set of equally spaced parallel grooves and on the other side a second set of equally spaced parallel grooves disposed at right angles to the first set, the first and second sets of grooves, respectively, of adjacent plates being in register with one another to provide two series of parallel passages traversing the block at right angles to one another.

One construction of heat exchanger made in accordance with this invention will now be described with reference to the accompanying drawings in which:

Figure 1 is a plan;

Figure 2 is a section on the line AA of Figure 1; and

Figure 3 is a section on the line BB of Figure 1;

50 The heat exchanger body proper is built up from a series of graphite plates 12 which are good heat conductors. Each plate 12 has on one side a first set of equally spaced parallel semi-cylindrical grooves 13 and on the other side a second set of equally spaced parallel semi-cylindrical grooves 14 lying in a direction at right angles to the direction of the first set 13, the alternate contiguous plate 12 being so arranged that the first sets of grooves lie in register with the first set of grooves in a contiguous plate and the second set of grooves in register with the second set of grooves in a contiguous plate so as to form first and second sets of cylindrical passages at right angles to one another. As shown in Figures 1 and 2 the passages formed by the grooves 14 open at their ends into the chambers 15 and 16 of cast iron headers 17 and 18. The header 18 is provided with steel inlet and outlet pipes 19 and 20 for the first fluid which in this case is a fluid which does not react with the iron or steel.

70 In the same way, as will be seen from Figure 3, the cylindrical passages formed by the semi-cylindrical grooves 13 open at their ends into headers 21 and 22 made of carbon. The hollow spaces 23 and the header 21 are sealed by glands 24, and similarly the hollow spaces 25 and the carbon header 22 are sealed by glands 26 and the carbon header 22 is provided with the carbon

inlet pipe 27 and a carbon outlet pipe 28 for the fluid which passes through the passages 13, which in this case is a fluid which might have a corrosive action or other reaction with metal. The graphite plates 12, which are good conductors of heat, conveniently have at the top and bottom thicker plates 29 of carbon with external cast iron cover plates 30. As shown in Figure 3 the carbon headers 21 and 22 have cast iron cover plates 31. The cover plates 30 and 31 are held in position by bolts 32 and nuts 33.

In the above described construction, the headers were of carbon or of cast iron and the cover plates were of cast iron. It is to be understood that other solid materials may be used for such headers and cover plates such as earthenware, vulcanised rubber, resin coated metal, artificial resin.

It is preferred to make each graphite plate by moulding from very finely pulverised coal with or without a small proportion of very finely divided pulverised coke or graphite and/or finely divided sulphur and after moulding to the required dimensions (allowing for subsequent shrinkage, e.g. 11% linear shrinkage) is embedded in coke fliers and fired under non-oxidising conditions to a temperature of 800 to 1000° C. at such a rate of temperature rise as to avoid intumescence as described in United States patent specification No. 2,461,365 or 2,493,383. Thereafter each plate is heated to a temperature of 2500° C. in an electric furnace. The conditions at this stage of the process are controlled in such a way that the carbon is not fully converted into graphite but into an intermediate form which has a high thermal conductivity (about 75% of that of natural graphite) but a higher strength and hardness than fully graphitised carbon.

Each plate is ground flat on each side in a grinding machine and each edge of each plate is ground straight and to the correct dimensions.

Grooves are formed in the plates by grinding, using a machine with a rotary grinding wheel the peripheral edge of which conforms to the shape of the groove required in the carbon plate. Thus for example when semi-cylindrical grooves are to be formed a grinding wheel having an edge of semi-circular section is employed.

There follow three examples of methods of manufacturing a low porosity carbon heat exchanger body in accordance with the invention, the body being substantially as shown in the drawings and made of 15 inch square graphite plates built up into a 15 inch cube, the bolts 32 for the cover plates each being of 1 inch diameter.

#### Example 1

(a) The graphite plates are assembled in the appropriate order, as set out above, to form a block.

(b) The cover plates 30 and 31 are positioned and the whole assembly subjected to a compressive load by the four bolts 32 connecting the cover plates. As set out hereinbefore, it is desirable that a compressive load shall be retained throughout the subsequent processing and a suitable torque loading on the bolts has been found to be at least 175 ft.-lbs.

(c) The assembly is dried to remove any residual moisture at a temperature of 125° C. for 2 hours.

(d) The assembly is placed in a suitable autoclave and a vacuum of at least 10 mm. of mercury absolute is applied for a period of 1 hour.

(e) A liquid mixture consisting of by weight, 90% cashew nut shell liquid and 10% diethyl sulphate as a polymerisation catalyst is prepared, the mixture being heated to 70° C. to reduce the viscosity into the range 30-40 centipoises.

(f) The resin mixture is then introduced into the autoclave in sufficient quantity to immerse the block completely with sufficient excess to allow a volumetric absorption of 30% of the volume of the graphite block.

(g) Air pressure of 50 lbs. per square inch is then applied within the autoclave for a period of 2 hours.

(h) The air pressure is released gradually over a period of about half an hour and the block is removed from the resin. The excess resin is allowed to drain from the block for a period of 12 hours.

(i) The assembly is placed in an oven, a slight internal air circulation being preferred, and is subjected to the following heating stages:

10 24 hours at 50° C.  
36 hours at 100° C.  
24 hours at 120° C.

(j) A slight porosity may still be present in the graphite due to the loss of the more volatile constituent of the resin during the polymerisation stage (i). Consequently a second impregnation is carried out using a resin of the following composition, by weight:

20 50% furfural  
50% furfuryl alcohol  
0.4 ccs. of N/1 H<sub>2</sub>SO<sub>4</sub> per lb. of mixture

A similar impregnation technique is carried out as in stages (d) to (i) with the following exceptions:

25 (1) The resin is used at room temperature (about 17° C.) and not pre-heated as the viscosity is low enough for the purpose required.

(2) The curing or polymerisation cycle (i) is modified to:

30 8 hours at 50° C.  
12 hours at 100° C.

(k) The torque loading is adjusted to 80 ft. lbs.

#### Example 2

35 (a) A cement mixture is prepared of the following composition:

92% cashew nut shell liquid  
8% para-formaldehyde

40 The resin should have a viscosity of 300 centipoises at 20° C.

(b) The cement is applied to the surfaces of the plates and the complete stack is assembled, the bottom cover plate being used as the base for that operation. It is preferred to use a jig to hold the plates in alignment whilst they are being stacked and the cement is preferably rolled on to the plates by means of a rubber roller.

(c) The top cover plate is placed in position and the four bolts are adjusted to hand tightness.

50 (d) The cement is allowed to pre-set for 12 hours at 20° C.

(e) The bolt loading is then adjusted to 80 ft.-lbs.

(f) The complete assembly is then heated at 80° C. for 12 hours to set the cement.

55 (g) Operations (d) to (k) of Example 1 are then performed.

#### Example 3

60 (a) Operations (a) to (f) of Example 2 are first carried out.

(b) A pair of cast iron headers are bolted to opposite faces of the block, a connection being provided in one header for the introduction of resin via a hand pump, and a connection being provided in the opposite header for draining resin from the block.

(c) Cashew nut shell resin mixture is prepared as described under (e) in Example 1 and is pumped into the headers via the hand pump until one set of cylindrical passages is filled with the mixture. Care should be taken to prevent air pockets forming.

(d) The pressure in the headers is raised to 50 lbs. per square inch and is held at this pressure until the resin exudes through the graphite plates to the other set of cylindrical passageways.

(e) The headers are removed and the unit allowed to drain for 12 hours.

(f) The curing cycle is then carried out as described under (i) in Example 1.

(g) A second vacuum impregnation is then carried out as described under (d) to (i) in Example 1.

(h) The torque on the bolts is then adjusted to 80 ft.-lbs.

After the final step in the above examples, the heat exchanger body is tested for the possibility of a leak. One pair of headers is bolted up and the header outlet is closed and the header inlet is subjected to substantial air pressure (e.g. 50 pounds per square inch), the body is immersed in water and is examined for any trace of air leak and in the event of a leak appearing re-impregnation is effected on the lines set out in any of the above examples.

Before impregnation in the above Examples 2 and 3, it is preferred that the faces of the block shall be machined flat to ensure close fitting of the headers. In the case of Example 1 the faces of the block are machined flat after impregnation and heat hardening.

I claim:

1. A method of manufacturing a low porosity carbon heat exchanger body comprising assembling a plurality of carbon plates to form a block, clamping said assembled plates together, said plates being grooved to provide passages traversing said block, and with the plates so assembled and clamped together impregnating the as-

sembled plates and therebetween with a liquid organic resin, and heat-hardening said resin to reduce the porosity of the plates and bond them together.

2. A method of manufacturing a low porosity carbon heat exchanger body comprising assembling a plurality of carbon plates to form a block, clamping said assembled plates together, each of said plates having on one side a first set of equally spaced parallel grooves and on the other side a second set of equally spaced parallel grooves disposed at right-angles to the first set, the first and second sets of grooves, respectively, of adjacent plates being in register with one another to provide two series of parallel passages traversing said block at right angles to one another, and with the plates so assembled and clamped together, impregnating the assembled plates and therebetween with a liquid organic resin, and heat-hardening said resin to reduce the porosity of said plates and bond them together.

#### References Cited in the file of this patent

##### UNITED STATES PATENTS

|           |                |               |
|-----------|----------------|---------------|
| 1,158,171 | Brown          | Oct. 26, 1915 |
| 1,834,895 | Brossman       | Dec. 1, 1931  |
| 2,247,355 | Brown          | July 1, 1941  |
| 2,512,230 | Greaves et al. | June 20, 1950 |
| 2,670,311 | Norman et al.  | Feb. 23, 1954 |

##### FOREIGN PATENTS

|         |               |              |
|---------|---------------|--------------|
| 620,998 | Great Britain | Apr. 1, 1949 |
|---------|---------------|--------------|